# EUROPEAN PATENT SPECIFICATION

(11) **EP 0 161 005 B1**
(45) Date of publication and mention of the grant of the patent: **20.12.1989**
(21) Application number: 85105887.5
(22) Date of filing: 13.05.1985
(51) Int. Cl.: C07C 91/40, G03C 1/72

(54) **Novel squarium compounds, process for preparing the same and electrophotographic photoreceptors containing the same**
"Squarium"-Verbindungen, Verfahren zu deren Herstellung und elekatrophotographische Photorezeptoren, die jene enthalten
Composés de "squarium", procédé de leur préparation et récepteurs électrophotographiques les contenant

(30) Priority: 11.05.1984 JP 92769/84; 11.05.1984 JP 92771/84
(43) Date of publication of application: 13.11.1985
(73) Proprietor: FUJI XEROX CO., LTD., Minato-ku Tokyo 107 (JP)
(72) Inventor: Saeki, Satoshi Fuji Xerox Co., Ltd., Minami Ashigara-shi Kanagawa (JP); Kin, Seki Fuji Xerox Co., Ltd., Minami Ashigara-shi Kanagawa (JP); Torikoshi, Kaoru Fuji Xerox Co., Ltd., Minami Ashigara-shi Kanagawa (JP); Tanaka, Hiroyuki Fuji Xerox Co., Ltd., Minami Ashigara-shi Kanagawa (JP); Sun Pu, Lyong Fuji Xerox Co., Ltd., Minami Ashigara-shi Kanagawa (JP)
(74) Representative: Boeters, Hans Dietrich, Dr.

(56) References cited:
- EP-A- 0 146 301
- US-A- 4 508 803
- CHEMICAL ABSTRACTS, vol. 100, no. 22. 28th May 1984, page 84, column 1, abstract no. 176464b, Columbus, Ohio, US

## Description

### Field of the Invention

This invention relates to novel squarium compounds having a flat photosensitivity in the wide range from visible ray region to the near infrared ray region as a charge generator, a process for preparing them and electrophotographic photoreceptors containing the squarium compounds.

### Background of the Invention

Hitherto, inorganic photographic materials such as amorphous selenium, selenium alloys, cadmium sulfide and zinc oxide and organic photographic materials represented by polyvinylcarbazole and polyvinylcarbazole derivatives are widely known as electrophotographic photoreceptors.

It is well known that amorphous selenium or selenium alloys have superior properties as electrophotographic photoreceptors and have been put into practice use. However, in producing these materials, a complicated vacuum deposition process is necessary, and further the vacuum-deposited film obtained has a disadvantage in that the film lacks flexibility. Zinc oxide is used as a dispersed photographic material in which zinc oxide is dispersed in a resin, but such material has a problem such as a low mechanical strength and cannot be used repeatedly as is.

Polyvinylcarbazoles known as organic photoconductive materials have advantages such as transparency, good film-forming property and flexibility, but polyvinylcarbazoles per se have no photosensitivity in at visible ray region, and cannot be used practically alone. Accordingly, various ' sensitization methods have been proposed therefor. Although a spectral sensitization of polyvinylcarbazole using a sensitizing dye has resulted in expanded spectral sensitivities extending to visible ray region, a sufficient photographic sensitivity as electrophotographic photoreceptors cannot be obtained, and it still has a drawback that a photo-fatigue is remarkable.

On the other hand, a spectral sensitization with an electron acceptor gives rise to electrophotographic photoreceptors having a sufficient photosensitivity, and some of them has been practically used. However, there is still more problems on mechanical strength and durability.

Various extensive studies have been made on photosensitive materials and there are many reports. However, electrophotographic photoreceptors having a superior electric characteristic and a sufficient photosensitivity have not yet been obtained. At present, there are reports about phthalocyanines which show superior electrophotographic characteristics as dispersed photosensitive materials. However, their spectral sensitivity is partial to long wavelength region, and they have a drawback that reproduction of red color is inferior.

### Summary of the Invention

An object of this invention is to provide novel squarium compounds having a flat photosensitivity in the wide range from the visible ray region to the near infrared ray region, a process for preparing squarium compounds and electrophotographic photoreceptors containing such squarium compounds.

Another object of this invention is to provide photoconductive materials having an extremely high photosensitivity, which are possible to use in every electrophotographic process and have a spectral sensitivity in the range from the visible ray region to the near infrared ray region.

A further object of this invention is to provide extremely superior electrophotographic photoreceptors having a flexibility that inorganic photographic materials fail to have, which are free from drawbacks of organic photographic materials such as polyvinylcarbazole-trinitrofluorenones, that is a low abrasion resistance and lack of mechanical strength, and which are superior in mechanical strength such as abrasion resistance and have a flat spectral sensitivity in the wide range from visible ray region to the near infrared ray region.

As a result of extensive studies to obtain photo-conductive materials having improved properties over conventional inorganic photographic materials, organic photographic materials or organic dispersed photographic materials, having superior electrophotographic properties and flexibility, and further having high photographic sensitivity in the wide range from visible ray region to the near infrared ray region, the present inventors found that the squarium compounds represented by the following general formula (I) possess extremely superior characteristics: wherein X represents a halogen atom, a nitro group, a cyano group, a formyl group, an acyl group, a carboxyl group or an alkoxycarbonyl group, n represents 0 or an integer of from 1 to 5, and R represents a hydrogen atom or a methyl group.

Relevant background art is described in CS-A-206 927 mentioning squarium compounds, the basic structure being m-toluidine. The known compounds are used as working substances of liquid lasers.

### Brief Description of the Drawings

Figures 1 and 2 are profile sections of compositions of electrophotographic photoreceptors of this invention.

In the figures, "1" shows an electroconductive support, "2" shows a charge generation layer, "3" shows a charge transport layer and "4" shows a photosensitive layer.

### Detailed Description of the Invention

The squarium compounds of this invention represented by formula (I) above can be prepared by reacting 3,4-dihydroxy-3-cyclobutene-1,2-dione (hereinafter referred to as squaric acid) represented by formula (II): with an aniline derivative of formula (III): wherein X, R and n have the same meanings as above.

In formulae (I), (II) and (III), the electron attractive group represented by X is a halogen atom, a nitro group, a cyano group, a formyl group, an acyl group, a carboxyl group or an alkoxycarbonyl group.

The reaction of squaric acid of formula (II) with an aniline derivative of formula (III) can be carried out by heating squaric acid and the aniline derivative in an inert organic solvent such as n-butyl alcohol or amyl alcohol at about 100°C to about 140°C for about 3 hours to about 5 hours. The resulting compound can be purified by washing and the recrystallizing the compound from an appropriate solvent.

Examples of the squarium compounds of formula (1) above of this invention include the following compounds.

The spectral sensitivity of the squarium compounds of this invention show a flat photosensitivity in the range of from 400 to 850 nm, and the squarium compounds of this invention have a sufficient photosensitivity in the range from the entire visible ray region to the near infrared ray region.

The squarium compounds of formula (I) can be used in electrophotographic photoreceptors having a multilayer structure. That is, in electrophotographic photoreceptors having a double layer structure consisting of a charge generation layer and a charge transport layer, a combination of the charge generation layer containing a squarium compound of this invention and a known charge transport layer comprising a photoconductive polymer such as a polyvinyldibenzothiaphene, a polyvinylpyrene, a polyvinylanthracene, a polyvinylcarbazole or a layer containing a triallylpyrazoline, a triphenylmethane, an oxadiazole, a tetraphenylbenzidine and a trinitrofluorenone, in a binder resin results in the improvement of chargibility of electrophotographic photoreceptors, lowering of residual potential, and further the improvement of mechanical strength.

As shown in Figures 1 and 2 which explain the construction of electrophotographic photoreceptor of this invention having a double layer structure, a photosensitive layer 4 which is composed of a lamination of charge generator layer 2 containing a squarium compound of this invention and a charge transport layer 3 containing a charge transport material is provided on an electroconductive support 1. The thickness ratio of the charge generation layer to the charge transport layer is preferably from about 1/2 to about 1/200. Further, the squarium compound and a charge transport material may be incorporated into one layer to form a single-layered photoreceptor, if desired.

The charge generation layer can consist of a squarium compound alone or a combination of the squarium compound and a binder resin. The ratio of the squarium compound of formula (I) to the binder resin used is from about 10% by weight to about 90% by weight, preferably from about 10% by weight to about 50% by weight.

A solvent coating method and a vacuum evaporation method can be used to prepare the charge generation layer with the squarium compound of this invention without using a binder resin.

The film thickness of charge generation layer is from about 0.1 u to about 3 u, preferably from 0.2 p to 1 µ.

For the purpose of its dispersion in a binder, the compound may be ground into fine particles by a known method using any conventional mill, such as an SPX MILL, ball mill or RED DEVIL (trade name). Particle size of the squarium compound is generally not more than 5 u, preferably 0.01 to 3 u, but the particle size is not limited thereto.

The binder used in the charge generation layer may have or may not have photoconductivity. Examples of binders having photoconductivity include photoconductive polymers such as polyvinylcarbazoles, polyvinylcarbazole derivatives, polyvinyl naphthalenes, polyvinylanthracenes, polyvinylpyrene, or other organic matrix materials having a charge transport property.

Moreover, known insulating resins which have not photoconductive property can be used as binders. Examples of such insulating resins include polystyrenes, polyesters, polyvinyltoluenes, polyvinylanisoles, polychlorostyrene, polyvinyl butyrals, polyvinyl acetate, polyvinylbutyl methacrylate, copolystyrene- butadiene, polysulfone, copolystyrenemethyl methacrylate and polycarbonate.

In order to improve mechanical strength of the electrophotographic photoreceptors obtained, a plasticizer can also be used as in the case of ordinary polymeric materials. Examples of plasticizers which can be used include chlorinated paraffin, chlorinated biphenyl, a phosphate plasticizer and a phthalate plasticizer. These plasticizers can be used in an amount of 0 to 10% by weight based on the weight of the binder used without adversely affecting the photosensitivity and electrical properties of the electrophotographic receptors thereby improving the mechanical properties.

The binder having dispersed therein a squarium compound is coated on an electroconductive support. The coating can be performed by a conventional method such as dip method, spray method, bar coater method and applicator method. A good photosensitive layer can be obtained by any of the above methods.

Usable electrically conductive supports include metals (e.g., aluminum, nickel, chromium, iron, stainless, copper, etc.), paper which is rendered electrically conductive, as well as polymeric films and glass plates having an electrically conductive coat of the above metals, Au, Ag, indium oxide, indium tin oxide, etc.

A surface layer such as a protective layer and an insulating layer may further be provided on the light-sensitive layer so as to prevent mechanical damage and chemical change in properties of the light-sensitive layer. The protective layer is a layer having low electric resistance of 10⁸ to 10¹⁴ Ωcm which can be used in so-called Carlson process, and the insulating layer is an electrically insulating layer which can be used in a process as described in U.S. Patents 3,041,167 and 3,438,706. Both layers are substantially transparent to light for exposure and the thicknesses of the protective layer and the insulating layer are about 2 to 20 p and about 10 to 40 µ, respectively.

In order to prevent injection of electron from an electrically conductive support to the light-sensitive layer, a barrier layer may be formed between the support and the light-sensitive layer. For the purpose, aluminum oxide, nylon, epoxy resins can be used. Such a barrier layer may not be formed when the photoreceptor is used in the process of U.S. Patents, 3,041,167 and 3,438,706 as described above or when the charge transport layer is formed as a lower layer on the support in the preparation of double-layered photoreceptor (Fig. 2). An adhesive layer may also be formed between the support and the light-sensitive layer to improve adhesion therebetween.

The electrophotographic photoreceptor of the present invention may be used not only with ordinary copiers but also with laser printers, as well as intelligent copiers since the photoreceptor of the present invention is sensitive to laser. Laser which can be applied to the photoreceptor of the present invention is preferably a semiconductor laser such as those of Ga-As type semiconductors (e.g., Ga-As, AI-Ga-As, Ga-As-P, etc.).

This invention will now be explained in more detail by the following examples.

### Example 1

### Preparation of Compound (I)

7.92 g of N-(4-fluorobenzyl)-N-methyl-m-toluidine and 2.0 g of squaric acid were heated in a mixture of n-butyl alcohol and toluene with stirring for 5 hours at 100°C to 120°C. After cooling, greenish crystals precipitated were collected by filtration and then washed with methanol to obtain 0.41 g (4.4% yield) of the desired squarium compound.
Decomposition point: 240°C to 241°C
Infrared absorption spectrum (KBr Tablet)
v C=O 1630 cm-¹
Visible absorption spectrum
λmax 647 nm (in dichloromethane solution)
Elemental analysis

### Examples 2 and 3

In the same manner as described in Example 1 but Compounds (4) and (6) were prepared.

### Compound (4)

Decomposition point: 232.5°C to 233.5°C
Infrared absorption spectrum (KBr Tablet)
v C=O 1590 cm-¹
Visible absorption spectrum
λmax 647 nm (in dichloromethane solution)
Elemental analysis

### Compound (6)

Decomposition point: 245.0°C to 245.5°C
Infrared absorption spectrum (KBr Tablet)
v C=O 1590 cₘ-¹
Visible absorption spectrum
λmax 639 nm (in dichloromethane solution)
Elemental analysis

### Example 4

The squarium compound wherein X is a 4-carboxyl group, n is 1 and R is a hydrogen atom was ground with dichloromethane and steel balls for 12 hours. The ground compound was then added to a polyester resin (Vylon 200, a tradename) in an amount of 30% by weight based on the weight of the polyester resin, followed by mixing, and then the mixture was coated by an applicator on an aluminum plate to prepare a charge generation layer having a thickness of about 0.5 µ (dry basis). A mixture of a polycarbonate resin (Panlite, a tradename) and 1-phenyl-3-[p-diethylaminostyryl]-5-[p-diethylaminophenyl]pyrazoline in an amount of 50% by weight based on the weight of the polycarbonate resin was then coated by an applicator on the charge generation layer to prepare a charge transport layer having thickness of about 15 µ.

The photosensitive surface of this photoreceptor was negatively charged with -6KV of corona electric discharge for 2 seconds using an electrostatic copy paper test instrument manufactured by Kawaguchi Denki Co., Ltd. After it was allowed to stand for 2 seconds in the dark, its surface potential (Vo) was measured and then a light from a tungsten-halogen lamp of illumination intensity of 10 lux was irradiated to the photosensitizer layer. The time when the value of the surface potential changed to a half the original value was determined to obtain a half value of exposure (E2). The results obtained were Vo of 655V and E½ of 6.5 lux-second.

### Examples 5 to 9

The electrophotographic photoreceptors of these examples were prepared in the same manner as described in Example 4 except that, each of the squarium compounds (2) to (6) shown in Table 1 was used, in place of the squarium compound used in Example 4. The electric characteristics of the resulting photoreceptors were determined, and the results obtained are shown in Table 1.

### Examples 10 to 15

Electrophotographic photoreceptors with inverted order of the charge generation layer and the charge transport layer were prepared in the same manner as those described in Examples 4 to 9 using squarium compounds (1) to (6) except that the order of the charge generation layer and the transport layer was inverted, and their electric characteristics were measured. The results obtained are shown in Table 2.

While the invention has been described in detail and with reference to specific embodiments thereof, it will be apparent to one skilled in the art that various changes and modifications can be made therein without departing from the spirit and scope thereof.

## Claims

1. A squarium compound represented by the general formula wherein X represents a halogen atom, a nitro group, a cyano group, a formyl group, an acyl group, a carboxyl group or an alkoxycarbonyl group, n = 0 or an integer of from 1 to 5 and R represents a hydrogen atom or a methyl group.

2. A squarium compound as claimed in Claim 1 represented by the general formula wherein X' represents a fluorine atom or a chlorine atom and Y represents a hydrogen atom or a fluorine atom.

3. A process for producing a squarium compound represented by the general formula wherein X, n and R have the same meanings as above, which comprises reacting 3,4-dihydroxy-3-cyclobutene-1,2-dione represented by the formula with an aniline derivative represented by the general formula, wherein X, n and R have the same meanings as above.

4. An electrophotographic photoreceptor comprising an electroconductive support and a light-sensitive layer comprising a squarium compound represented by the formula wherein X represents a halogen atom, a nitro group, a cyano group, a formyl group, an acyl group, a carboxyl group or an alkoxycarbonyl group, n is 0 or an integer of from 1 to 5 and R represents a hydrogen atom or a methyl group.

5. The photoreceptor claimed in claim 4, wherein said light-sensitive layer comprises a charge transport layer and a charge generation layer containing said squarium compound.

6. The photoreceptor claimed in claim 5, wherein said charge transport layer comprises a photo- conductive polymer selected from the group consisting of poly(vinyldibenzothiophene), poly(vinylpyrene), poly(vinylanthracene) and poly(vinylcarbazole).

7. The photoreceptor claimed in claim 5, wherein said charge transport layer comprises triallylpyrazoline, triphenylmethane, oxadiazole, tetraphenylbenzidine or trinitrofluorenone and a binder resin.

8. The photoreceptor claimed in claim 5, wherein said charge generation layer is comprised substantially of said squarium compound.

9. The photoreceptor claimed in claim 5, wherein said charge generation layer comprises said squarium compound in an amount of from about 10 to 90 weight percent based on the weight of the charge generation layer.

10. The photoreceptor claimed in claim 9, wherein said squarium compound is present in an amount of from about 10 to 50 weight percent based on the weight of the charge generation layer.

11. The photoreceptor claimed in claim 5, wherein said charge generation layer is from about 0.1 to 3 micron thick.

12. The photoreceptor claimed in claim 11, wherein the thickness ratio of said charge generation layer to said charge transport layer is from about 1/2 to about 1/200.

13. The photoreceptor claimed in claim 5, wherein said charge generation layer is between said support and said charge transport layer.

14. The photoreceptor claimed in claim 7, wherein said charge transport layer is between said support and said charge generation layer.

15. The photoreceptor claimed in claim 4, wherein said light-sensitive layer comprises a layer containing said squarium compound and a charge transport material.

16. The photoreceptor claimed in claim 5, wherein said squarium compound is dispersed in the form of particles in said charge generation layer.

## Patentansprüche

1. Eine Squariumverbindung der allgemeinen Formel worin X ein Halogenatom, eine Nitrogruppe, eine Cyanogruppe, eine Formylgruppe, eine Acylgruppe, eine Carboxylgruppe oder eine Alkoxycarbonylgruppe darstellt, n = 0 oder eine ganze Zahl von 1 bis 5 ist und R ein Wasserstoffatom oder eine Methylgruppe darstellt.

2. Squariumverbindung nach Anspruch 1, der allgemeinen Formel worin X' ein Fluoratom oder ein Chloratom und Y ein Wasserstoffatom oder ein Fluoratom bedeuten.

3. Verfahren zur Herstellung einer Squariumverbindung der allgemeinen Formel worin X, n und R die vorstehend angegebenen Bedeutungen besitzen, bei dem man 3,4-Dihydroxy-3-cyclo- buten-1,2-dion der allgemeinen Formel mit einem Anilinderivat der allgemeinen Formel umsetzt, worin X, n und R die vorstehend angegebenen Bedeutungen besitzen.

4. Elektrophotografischer Photorezeptor mit einem elektrisch leitenden Träger und einer lichtsensitiven Schicht mit einer Squariumverbindung der Formel worin X ein Halogenatom, eine Nitrogruppe, eine Cyanogruppe, eine Formylgruppe, eine Acylgruppe, eine Carboxylgruppe oder eine Alkoxycarbonylgruppe bedeutet, n = 0 oder eine ganze Zahl von 1 bis 5 ist und R ein Wasserstoffatom oder eine Methylgruppe bedeutet.

5. Photorezeptor nach Anspruch 4, bei dem die lichtempfindliche Schicht eine Ladungstransportschicht und eine Ladungserzeugungsschicht mit einem Gahalt an der Squariumverbindung umfaßt.

6. Photorezeptor nach Anspruch 5, bei dem die Ladungstransportschicht ein photoleitendes Polymeres aus der aus Poly-(vinyldibenzothiophen), Poly-(vinylpyren), Poly-(vinylanthracen) und Poly-(vinylcarbazol) gebildeten Gruppe umfaßt.

7. Photorezeptor nach Anspruch 5, bei dem die Ladungstransportschicht Triallylpyrazolin, Triphenylmethan, Oxadiazol, Tetraphenylbenziden oder Trinitrofluorenon und ein Bindemittelharz umfaßt.

8. Photorezeptor nach Anspruch 5, bei dem die Ladungserzegungsschicht im wesentlichen aus der Squariumverbindung besteht.

9. Photorezeptor nach Anspruch 5, bei dem die Ladungserzeuzeugungsschicht die Squariumverbindung in einer Menge von etwa 10 bis 90 Gew.-% auf Basis des Gewichts der Ladungserzeugungsschicht umfaßt.

10. Photorezeptor nach Anspruch 9, bei dem die Squariumverbindung in einer Menge von etwa 10 bis 50 Gew-% auf Basis der Gewichts der Ladungserzeugungsschicht vorliegt.

11. Photorezeptor nach Anspruch 5, bei dem die Ladungserzeugungsschicht etwa 0,1 bis 3 um dick ist.

12. Photorezeptor nach Anspruch 11, bei dem das Dickenverhältnis der Ladungserzeugungsschicht zur Ladungstransportschicht etwa 1/2 bis etwa 1/200 beträgt.

13. Photorezeptor nach Anspruch 5, bei dem die Ladungserzeugungsschicht zwischen dem Träger und der Ladungstransportschicht angeordnet ist.

14. Photorezeptor nach Anspruch 7, bei dem die Ladungstransportschicht zwischen dem Träger und der Ladungserzeugungsschicht angeordnet ist.

15. Photorezeptor nach Anspruch 4, bei dem die lichtempfindliche Schicht eine Schicht umfaßt, die die Squariumverbindung und ein Ladungstransportmaterial enthält.

16. Photorezeptor nach Anspruch 5, bei dem die Squariumverbindung in Form von Teilchen in der Ladungserzeugungsschicht dispergiert ist.

## Revendications

1. Un composé squarium de formule générale I ci-dessous: dans laquelle X représente un atome d'halogène ou un groupe nitro, cyano, formyle, acyle, carboxyle ou alcoxycarbonyle, n un entier de 0 à 5 et R un atome d'hydrogène ou le groupe méthyle.

2. Un composé squarium de la revendication 1, de formule générale ci-dessous: dans laquelle X' représente un atome de fluor ou de chlore et Y un atome d'hydrogène ou de fluor.

3. Un procédé de production d'un composé squarium de formule générale: dans laquelle X, n et R ont la même signification que ci-dessus, procédé selon lequel on fait réagir une 3,4-dihydroxy-3-cyclobutène-1,2 dione de formule: avec un dérivé d'aniline de formule générale: dans laquelle X, n et R ont la même signification que ci-dessus.

4. Un photorécepteur électrophotographique comprenant un support électroconducteur et une couche photosensible qui comprend un composé squarium de formule: dans laquelle X représente un atome d'halogène ou un groupe nitro, cyano, formyle, acyle, carboxyle ou alcoxycarbonyle, n un entier de 0 à 5 et R un atome d'hydrogène ou le groupe méthyle.

5. Le photorécepteur de la revendication 4 dans lequel la couche photosensible comprend une couche de transport de charges et une couche de production de charges contenant ce composé squarium.

6. Le photorécepteur de la revendication 5 dans lequel la couche de transport de charges comprend un polymère photoconducteur choisi parmi un poly-(vinyldibenzothiophène), un poly-(vinylpyrène), un poly-(vinylanthracène) et un poly-(vinylcarbazole).

7. Le photorécepteur de la revendication 5 dans lequel la couche de transport de charges comprend de la triallylpyrazoline, du triphénylméthane, de l'oxadiazole, de la tétraphénylbenzidine ou de la trinitro- fluorénone avec une résine comme liant.

8. Le photorécepteur de la revendication 5 dans lequel la couche de production de charges est essentiellement formée du composé squarium.

9. Le photorécepteur de la revendication 5 dans lequel la couche de production de charges comprend le composé squarium dans une proportion d'environ 10 à 90% en poids par rapport au poids de cette couche.

10. Le photorécepteur de la revendication 9 dans lequel la proportion du composé squarium est d'environ 10 à 50% du poids de la couche de production de charges.

11. Le photorécepteur de la revendication 5 dans lequel la couche de production de charges a une épaisseur d'environ 0,1 à 3 microns.

12. Le photorécepteur de la revendication 11 dans lequel le rapport de l'épaisseur de la couche de production de charges à l'épaisseur de la couche de transport de charges est compris entre environ 1/2 et 1/200.

13. Le photorécepteur de la revendication 5 dans lequel la couche de production de charges est disposée entre le support et la couche de transport de charges.

14. Le photorécepteur de la revendication 7 dans lequel la couche de transport de charges est disposée entre le support et la couche de production de charges.

15. Le photorécepteur de la revendication 4 dans lequel la couche photosensible comprend une couche contenant le composé squarium et une matière de transport de charges.

16. Le photorécepteur de la revendication 5 dans lequel le composé squarium est dispersé en particules dans la couche de production de charges.
